

## UNITED STATES PATENT OFFICE

2,604,399

PHOTOGRAPHIC DEVELOPERS COMPRISING  
BIS-(DI-HYDROXYALKYL AMINOMETHYL)-HYDROQUINONES

Thomas S. Donovan and Frederic R. Bean, Rochester, N. Y., assignors to Eastman Kodak Company, Rochester, N. Y., a corporation of New Jersey

No Drawing. Application July 7, 1949,  
Serial No. 103,532

12 Claims. (Cl. 95—88)

1

This invention relates to photographic developers and more particularly to photographic developing solutions.

Prominent among the developing agents now employed in the rapid development of photographic images are those comprising hydroquinone and Elon (p-N-methylaminophenol). While various formulas of these developers are excellently suited for general photographic use, they have not been outstanding where developers of increased water solubility are required. For example, certain aqueous photographic developer solutions comprising hydroquinone and Elon give rise to the formation of a precipitate after the solutions have been allowed to stand for a time.

Photographic developers which possess this desired water solubility would represent a substantial advance in the art, if such developers retained much of the developing activity exercised by hydroquinone.

It is, therefore, an object of our invention to provide photographic developers which possess water solubility of a high degree. A further object is to provide photographic developers which, in addition to having a high degree of water solubility, have sufficient developing activity (ability to reduce silver halide) to warrant their use in developing solutions. Other objects will become apparent from the following description and examples.

According to our invention we accomplish the above objects by providing photographic developer solutions comprising a bis-[di-(hydroxyalkyl)aminomethyl]hydroquinone.

The bis-[di-(hydroxyalkyl)aminomethyl]hydroquinones useful in practicing our invention can advantageously be represented by the following general formula:



wherein R and R<sub>1</sub> each represents a hydroxyalkyl group containing from 2 to 3 carbon atoms. Compounds represented by the above formula which have been found to be especially

useful for the purposes of our invention include those represented by the following formulas:



30 The compounds represented by the above formulas can be used either in the form of their free base or in the form of an acid addition salt thereof (e. g. oxalate, sulfate, acetate, etc.). The free bases of the above compounds are soluble in water, we have found.

The following is an example of a standard photographic developer formula useful in practicing our invention:

40

## EXAMPLE 1

|                                                                       |            |
|-----------------------------------------------------------------------|------------|
| Elon (p-(N-methylamino)phenol) grams                                  | 2.5        |
| 2,5-bis-[di-( $\beta$ -hydroxyethyl)aminomethyl]-hydroquinone oxalate | 2.5        |
| Sodium sulfite (anhydrous)                                            | 75.0       |
| Sodium carbonate (anhydrous)                                          | 25.0       |
| Potassium bromide                                                     | 1.5        |
| Water to                                                              | 1.0 liters |

This developer solution was used to develop motion-picture positive film.

## EXAMPLE 2

Another formula which has been found useful in practicing our invention is:

|                                                    |                     |       |     |
|----------------------------------------------------|---------------------|-------|-----|
| 2,5-bis-[di-( $\beta$ -hydroxyethyl) aminomethyl]- | hydroquinone oxlate | grams | 5.0 |
| Sodium sulfite (anhydrous)                         | do                  | 75.0  |     |
| Sodium carbonate (anhydrous)                       | do                  | 25.0  |     |
| Potassium bromide                                  | do                  | 1.5   |     |
| Water to                                           | liters              | 1.0   |     |

Photographic developer formulas other than those illustrated above can be employed to advantage. Both the amount and type of hydroquinone developing agent can be varied to suit the requirements of the operator. The above formulas are merely illustrative and are not intended to limit our invention.

The developing agents represented by the above general formula are especially useful in the preparation of concentrated photographic developer formulas which find use in the field of X-ray photography. The developers coming within the scope of the present invention are characterized by their excellent solubility in water, a property which is much desired for such concentrated photographic formulas. Whereas the conventional HQ-MQ (hydroquinone-Elon) concentrated developer solutions give rise to precipitates on standing, the developer solutions of the present invention do not show a precipitate at even higher concentrations. Typical concentrated developer formulas in which the hydroquinone compounds of our invention can be used include those illustrated in the application of F. R. Bean, Serial No. 94,510, filed May 20, 1949, now U. S. Patent 2,578,281, issued December 11, 1951. Such solutions generally comprise from about 50 to 75 grams of phenolic developer per liter of solution, although many of the hydroquinone compounds of our invention permit even higher concentrations of phenolic developers to be used. The hydroquinone compounds represented by the above general formula can also be used in tanning developer solutions, although usually less efficaciously than hydroquinone itself, we have found.

The following examples illustrate the method of preparation of typical hydroquinone compounds coming within the scope of our invention.

## EXAMPLE 3

2,5 - bis[di-( $\beta$ -hydroxyethylamino) ethyl]hydroquinone oxalate

55 g. of hydroquinone were dissolved in 125 cc. of water and 105 g. of diethanolamine were added. The solution was cooled to 15° C., 87 cc. of a 37 per cent formalin solution were added dropwise with stirring over a period of 30 minutes, and the solution was then stirred at room temperature for an additional hour. The reaction mixture was concentrated under a vacuum to a thin syrup, 500 cc. of acetone added, and the acetone solution made acid to Congo Red with oxalic acid. The product crystallized as fine, white prisms melting at 196°-197° C. (with decomposition). They were very soluble in water.

## EXAMPLE 4

2,5-bis - [di-( $\beta$  - hydroxyisopropyl) aminomethyl] hydroquinone

28 g. of hydroquinone were dissolved in 125 cc. of a 75% solution of ethyl alcohol, and 77 g. of diisopropanolamine were added. The solu-

tion was cooled to 15° C., and 44 cc. of 37 per cent formalin were added dropwise with stirring. The mixture was then warmed on a steam bath for 30 minutes and the alcohol removed by evaporation. The syrupy residue was taken up in 150 cc. of water, the solution treated with decolorizing carbon and filtered. From the filtrate, on standing, there separated a tan crystalline solid which was recrystallized from ethanol. The crystals melted at 180°-182° C. and were soluble in water, acids, alkalies, and alcohol. They were essentially insoluble in ether or benzene.

Other hydroquinone compounds useful in practicing our invention can be prepared by interacting hydroquinone, formaldehyde and other hydroalkylamines in the manner described above.

The hydroquinone compounds of our invention can be mixed with the usual strongly alkaline materials employed in photographic developer solutions to give a dry mixture, and this mixture can then be dissolved in water to give a solution useful in preparing the desired developing formulas, i. e. the usual constituents employed in photographic formulas can then be added. The ratio of materials added to the mixture correspond to those given in the above formulas, although other known ratios of developing agent to alkali can be used to advantage, as set forth above, the particular ratios desired can be varied to suit the requirements of the operator.

The bis-[di - (hydroxyalkyl) aminomethyl]hydroquinones of our invention can also be used as oxidation inhibitors for gasoline, fatty oils, rubber, resins, etc. They can also be efficaciously used in processes for oxidatively dyeing wool or fur, e. g. in the form of their dilute aqueous alkaline solutions (or by soaking the object to be dyed in an alcoholic solution of the hydroquinone compound) and then exposing to air or the influence of oxidizing agents, such as hydrogen peroxide. Mordants (e. g. ferrous sulfate, copper sulfate, sodium dichromate, etc.) can be used.

What we claim as our invention and desire secured by Letters Patent of the United States is:

1. A photographic silver halide developer solution comprising as the active developing agent an acid addition salt of a compound selected from those represented by the following general formula:



wherein R and R<sub>1</sub> represents a hydroxyalkyl group.

2. A photographic silver halide developer solution comprising as the active developing agent an acid addition salt of a compound selected from those represented by the following general formula:



wherein R and R<sub>1</sub> each represents a hydroxalkyl group containing from 2 to 3 carbon atoms.

3. A photographic silver halide developer solution comprising as the active developing agent an acid addition salt of a compound selected from those represented by the following general formula:



wherein R and R1 each represents a  $\beta$ -hydroxyalkyl group containing from 2 to 3 carbon atoms.

4. A photographic silver halide developer solution comprising as the active developing agent an acid addition salt of the compound represented by the following formula:



5. A photographic silver halide developer solution comprising as the active developing agent an acid addition salt of the compound represented by the following formula:



6. A photographic silver halide developer solution comprising as the active developing agent an acid addition salt of the compound represented by the following formula:



7. A solid mixture of chemicals useful for forming a photographic silver halide developer solution by dissolving in water comprising as a developing agent an acid addition salt of a compound selected from those represented by the following general formula:



wherein R and R1 each represents a hydroxyalkyl group, and a strongly alkaline material.

8. A solid mixture of chemicals useful for forming a photographic silver halide developer solution by dissolving in water comprising as a developing agent an acid addition salt of a compound selected from those represented by the following general formula:



wherein R and R1 each represents a hydroxyalkyl group containing from 2 to 3 carbon atoms, and a strongly alkaline material.

9. A solid mixture of chemicals useful for forming a photographic silver halide developer solution by dissolving in water comprising as a developing agent an acid addition salt of a compound selected from those represented by the following general formula:



wherein R and R1 each represents a hydroxyalkyl group containing from 2 to 3 carbon atoms, and a strongly alkaline material.

10. A solid mixture of chemicals useful for forming a photographic silver halide developer solution by dissolving in water comprising as a developing agent an acid addition salt of the compound represented by the following formula:



and a strongly alkaline material.

11. A solid mixture of chemicals useful for forming a photographic silver halide developer solution by dissolving in water comprising as a developing agent an acid addition salt of the compound represented by the following formula:



and a strongly alkaline material.

12. A solid mixture of chemicals useful for forming a photographic silver halide developer solution by dissolving in water comprising as a developing agent an acid addition salt of the compound represented by the following formula:



and a strongly alkaline material.

THOMAS S. DONOVAN.  
FREDERIC R. BEAN.

(References on following page)

## REFERENCES CITED

The following references are of record in the file of this patent:

## UNITED STATES PATENTS

| Number    | Name            | Date          |
|-----------|-----------------|---------------|
| 2,163,166 | Wilmanns et al. | June 20, 1939 |
| 2,304,953 | Peterson        | Dec. 15, 1942 |

5

## OTHER REFERENCES

Henney and Dudley, "Handbook of Photography," McGraw-Hill, New York, 1939; pages 328, 329, and 334 cited.